

2,982,734

## POWER TRANSMISSION MINERAL OIL BASE FLUID

Stanley R. Sprague, East Alton, and Theodore W. Havelly, Alton, Ill., assignors to Shell Oil Company, a corporation of Delaware

No Drawing. Filed June 14, 1957, Ser. No. 665,659

3 Claims. (Cl. 252—78)

This invention pertains to improved functional fluids having good lubricating properties. More particularly this invention relates to mineral oil compositions for use in an apparatus by means of which mechanical forces are transmitted or absorbed such as in automotive and truck transmissions, hydraulic brakes, clutches and various other mechanical equipment.

The smooth functioning of various power transmitting mechanisms, particularly the more complicated automotive transmissions, fluid-cooled brake mechanisms and the like, oil lubricated wet clutches, planetary gears and hydraulic control mechanisms, depend on adequate cooling and lubricating of the equipment. Rigorous requirements have been set up to qualify fluids for this service which includes wide temperature stability at both high and low temperatures and a low pour point to insure proper pumpability and fluidity at low temperatures. The fluids must not have a detrimental effect on parts with which they come in contact, such as metal surfaces, e.g., copper, and solid non-metallic surfaces, such as organic resins and the like. They must possess excellent antifrictional and, in some cases extreme pressure characteristics, to afford proper lubrication of gears, clutch plates and other parts of the mechanism in which they are used, such as automotive equipment. Also the fluids must not cause chattering, squawking, squealing or produce other noises caused by the frictional vibrations and/or stick-slip phenomenon of clutch plates or other parts of such mechanisms.

The prior art discloses various functional or power transmission fluids of the mineral oil or synthetic oil type (organic esters and polyethers) containing as the improving agents various organic phosphates, fatty acids and their esters, halogenated compounds, polymers such as polyacrylates and the like. Compositions of this type are objectionable because of their inability to eliminate chattering and noises caused by frictional vibrations and/or stick-slip phenomenon of clutch plates and the like, particularly in equipment which is subjected to high speeds and temperatures.

The present invention is based on the discovery that certain combinations of materials are highly effective for the above purpose in small amounts of from about 0.01% to about 5%, preferably from about 0.1% to about 1%, by weight, in a hydrocarbon oil of wide viscosity range.

The agents are respectively saturated fatty acids having from 18 to 30 carbon atoms and preferably saturated fatty acids having from 18 to 26 carbon atoms, such as stearic acid and cerotic acid and mono- or di-aliphatic acid phosphates such as mono- or di-saturated or unsaturated alkyl acid phosphates e.g., mono- or di-alkyl acid phosphate, or mono- or di-alkenyl phosphates or mixtures thereof, said alkyl or alkenyl radicals having at least 9 carbon atoms and preferably at least 18 and up to 36 carbon atoms in the aliphatic group. Examples of suitable mono- and di-acid phosphates are dilauryl acid

phosphate, distearyl acid phosphate, dibehenyl acid phosphate, distearyl acid phosphate, dioleyl acid phosphate, lauryl diacid phosphate, stearyl diacid phosphate, behenyl diacid phosphate, oleyl diacid phosphate, and mixtures 5 thereof such as mono and dilauryl acid phosphate, mono and distearyl acid phosphate, mono and distearyl acid phosphate and the like.

In addition to the above two essential additives and mixtures thereof it is preferred to use in such compositions small amounts of from about 0.01% to about 1% of phenolic, amine and/or metal thiophosphate antioxidants such as alkyl phenols, e.g., di- and trialkyl phenols, for instance 2,4-, 2,3-, 3,4-, 2,6- and 3,5-diamyl phenol, 2,4-dimethyl-6-tertbutyl phenol, 2,6-ditertbutyl-14-methyl phenol; arylamines such as phenyl- $\alpha$ -naphthyl-amine or phenyl- $\beta$ -naphthyl-amine; metal thiophosphates such as calcium or zinc dimethyl cyclohexylidithiophosphate anti-foaming agent e.g., silicone polymers (DC 200 fluids ranging in viscosity in centistokes from 100 to 1000 at 250° C.) or Silicone type A fluid made by Dow-Corning Co. and described in U.S. Patents 2,563,588 and 2,662,055 and mixtures thereof.

As stated above the base oils are hydrocarbon oils of wide viscosity range. Such oils have a viscosity in the range of 40 SUS at 100° F. to 150 SUS at 210° F. and are illustrated by mineral oils which include mineral spirits, mineral seal oil, mineral spray oil transformer oil as well as lubricating oils having SAE numbers of from SAE 10 to SAE 50. Illustrative oils of this type have 30 the following properties:

### SAE 10 MINERAL OIL

|                          |      |
|--------------------------|------|
| Viscosity SUS at 100° F. | 175  |
| Viscosity SUS at 210° F. | 45.2 |
| Viscosity index          | 106  |
| Flash, ° F.              | 395  |
| Fire, ° F.               | 440  |
| Pour point, ° F.         | —35  |

40 Another suitable base oil is a highly refined transformer oil (A) having the following properties:

|                          |           |
|--------------------------|-----------|
| GR. ° API                | 30.9      |
| Color                    | 30        |
| Viscosity SUS at 100° F. | 56.9      |
| Flash, COC, ° F.         | 290       |
| Fire, COC, ° F.          | 320       |
| Pour point, ° F.         | below —70 |

50 Still another suitable base oil is a refined oil (B) having the following properties:

|                          |      |
|--------------------------|------|
| GR. ° API                | 31.2 |
| Color ASTM               | —1   |
| Pour point               | —30  |
| Flash, ° F.              | 270  |
| Fire, ° F.               | 295  |
| Viscosity SUS at 100° F. | 48   |
| Viscosity index          | 33   |

60 The following compositions are illustrative of the invention:

|                              | Composition A | Weight percent |
|------------------------------|---------------|----------------|
| Monostearyl diacid phosphate | 0.05          |                |
| Stearic acid                 | 0.2           |                |
| Mineral oil (B)              | Balance       |                |

|                              | Composition B | Weight percent |
|------------------------------|---------------|----------------|
| Monohehenyl diacid phosphate | 0.05          |                |
| Stearic acid                 | 0.02          |                |
| Mineral oil (A)              | Balance       |                |

| Composition C               |                |
|-----------------------------|----------------|
|                             | Weight percent |
| Monolauryl diacid phosphate | 0.2            |
| Stearic acid                | 0.2            |
| Mineral oil (B)             | Balance        |

| Composition D             |                |
|---------------------------|----------------|
|                           | Weight percent |
| Monolauryl acid phosphate | 0.1            |
| Stearic acid              | 0.2            |
| Mineral oil (SAE 10)      | Balance        |

| Composition E                               |                |
|---------------------------------------------|----------------|
|                                             | Weight percent |
| Mixture of mono and dilauryl acid phosphate | 0.1            |
| Stearic acid                                | 0.2            |
| Mineral oil (B)                             | Balance        |

| Composition F                   |                |
|---------------------------------|----------------|
|                                 | Weight percent |
| Monostearyl diacid phosphate    | 0.1            |
| Stearic acid                    | 0.2            |
| 2,6-ditertbutyl-4-methyl phenol | 0.2            |
| Phenyl- $\alpha$ -naphthylamine | 0.1            |
| Mineral oil (B)                 | Balance        |

| Composition G                |                |
|------------------------------|----------------|
|                              | Weight percent |
| Monobehenyl diacid phosphate | 0.1            |
| Cerotic acid                 | 0.2            |
| Mineral oil (SAE 10)         | Balance        |

| Composition H                       |                |
|-------------------------------------|----------------|
|                                     | Weight percent |
| Mono-oleyl diacid phosphate         | 0.3            |
| Stearic acid                        | 0.2            |
| 2,6-ditertbutyl-4-methyl phenol     | 0.2            |
| Phenol- $\alpha$ -naphthylamine     | 0.1            |
| D-C 200 Fluid* (1000 cs. at 25° C.) | 5 p.p.m.       |
| Mineral oil (A)                     | Balance        |

\*D-C 200 Fluid = dimethyl silicone polymer.

The superiority of compositions of this invention to eliminate noise, frictional vibrations and stick-slip sliding in liquid cooled hydraulic brake systems in which the parts were made of steel and resilient, or semi-metallic, or full sintered metallic friction materials were evaluated in actual automobile tests wherein the noise created after accelerating and suddenly stopping the vehicle was rated,

10 being excellent, no noise or stick-slip and zero (0) being poor, severe noise and stick-slip.

With compositions A, B, C, D, E, F, G and H the ratings were between 8 and 10. Mineral oils (A) or (B) each containing 0.2% stearic acid or 0.2% cerotic acid gave ratings of 4 and 5 respectively. Mineral oil (A) or (B) each containing 0.5% of n-octyl acid phosphate, di-octyl acid phosphate and triisooctyl phosphate, gave ratings of 4.1 and 1 respectively, while mineral oil (A) containing 0.4% lauryl acid phosphate gave a rating of 3.

Additives of this invention are useful in various functional fluids which contain minor amounts of other agents such as viscosity index improvers, point depressants, corrosion inhibitors and the like.

We claim as our invention:

1. A power transmission fluid consisting essentially of a major amount of mineral oil containing from about 0.1% to about 1% stearic acid, from about 0.01% to about 1% ditertbutyl-4-methylphenol, from about 0.01% to about 1% phenyl-alpha-naphthylamine and from about 0.1% to about 1% of diacid phosphate selected from the group consisting of monooleyl diacid phosphate and monostearyl diacid phosphate.

2. A power transmission fluid consisting essentially of a major amount of mineral lubricating oil and containing 0.2% stearic acid, 0.3% mono-oleyl diacid phosphate, 0.2% 2,6-ditertbutyl-4-methyl phenol and 0.1% phenyl- $\alpha$ -naphthylamine.

3. A power transmission fluid consisting essentially of a major amount of mineral lubricating oil and containing 0.2% stearic acid, 0.3% monostearyl diacid phosphate, 0.2% 2,6-ditertbutyl-4-methyl phenol and 0.1% phenyl- $\alpha$ -naphthylamine.

#### References Cited in the file of this patent

#### UNITED STATES PATENTS

|           |               |               |
|-----------|---------------|---------------|
| 2,005,619 | Graves        | June 18, 1935 |
| 2,080,299 | Benning       | May 11, 1937  |
| 2,203,102 | Powers        | June 4, 1940  |
| 2,447,483 | Baker         | Aug. 24, 1948 |
| 2,686,760 | Watson        | Aug. 17, 1954 |
| 2,687,377 | Stewart       | Aug. 24, 1954 |
| 2,694,045 | Jones         | Nov. 9, 1954  |
| 2,779,739 | Spivak        | Jan. 29, 1957 |
| 2,830,956 | Wasson et al. | Apr. 15, 1958 |
| 2,913,415 | Schmitz       | Nov. 17, 1959 |